

1

3,389,959

MANUFACTURE OF TRIPLE SUPERPHOSPHATE  
Donald E. Lee, Atlanta, Ga., assignor, by mesne assignments, to Armour Agricultural Chemical Company, a corporation of Delaware  
No Drawing. Filed Apr. 30, 1965, Ser. No. 452,347  
5 3 Claims. (Cl. 23—109)

ABSTRACT OF THE DISCLOSURE

Triple superphosphate is prepared by acidulating low-grade phosphate ore having less than 62 BPL with wet process superphosphoric acid having at least 65 weight percent  $P_2O_5$  equivalent and at a  $P_2O_5/CaO$  ratio of about 1.0 to 1.1, and heating the mixture to a temperature in the range of about 250–450° F., and storing the heated mass for reaction to form triple superphosphate. While the superphosphoric acid may be mixed with the phosphate rock at room temperatures, the superphosphoric acid is preferably heated to about 250–450° F. and then mixed with the rock and the mixture then heated to 250–450° F. before being stored in a den for reaction to form triple superphosphate.

This invention relates to the manufacture of triple superphosphate and more particularly to the beneficiation of low grade phosphate rock or ore through the production process.

An object of the invention is to provide for the production of triple superphosphate from low grade phosphate rock which has heretofore been considered unsuitable for triple superphosphate production. Another object is to provide a process in which superphosphoric acid is employed effectively for the beneficiation of low grade phosphate ore or rock and to produce triple superphosphate of substantially greater than 46%  $P_2O_5$  analysis. Yet another object is to provide a process employing effective  $P_2O_5/CaO$  ratios and initial heating steps by which triple superphosphate is produced having a relatively high  $P_2O_5$  analysis from low grade phosphate of less than 62 BPL. Other specific objects and advantages will appear as the specification proceeds.

In one embodiment of the invention a low grade phosphate rock of less than 62 BPL is treated with wet process superphosphoric acid having at least 65%  $P_2O_5$  weight percent and thereafter the mixture is stored in a den, as in a conventional triple superphosphate process, for reaction to form a triple superphosphate product.

In the foregoing process, I employ a  $P_2O_5/CaO$  ratio of 0.9 to 1.1, the ratio of 1.0 or 1.1 being preferred. While

2

The oven heating step may be for any suitable period but ordinarily 30 minutes is a sufficient time for such heating.

Specific examples illustrative of the process may be set out as follows:

EXAMPLE I

A low grade phosphate rock (61.4 BPL), which heretofore has been considered unsuitable for triple superphosphate production, was mixed with 65 weight percent  $P_2O_5$  wet process superphosphoric acid. The phosphate rock was from Bartow, Fla., and contained 0.18%  $H_2O$ , 40.15%  $CaO$ , 28.10%  $P_2O_5$  and 3.40% fluorine. The wet process phosphoric acid had a total  $P_2O_5$  of 72.0%, an ortho phosphoric acid content of 38.5%  $P_2O_5$ , and a fluorine content of 0.29%.

The reaction conditions are set out as follows:

| 20 |      | Initial Temp., ° F. |       |                |
|----|------|---------------------|-------|----------------|
|    |      | No. 1               | No. 2 | No. 3          |
|    |      | Rock                | Room  | 110            |
|    | Acid | 150                 | 170   | 180            |
|    |      |                     |       | Set Time, sec. |
| 25 |      |                     |       |                |
|    | Den  | 50                  | 37    | 40             |

The product analysis is set out in the following table:

TABLE I

| 30 |                                     | No. 1          |                            |                                    | No. 2                  |                                |                   | No. 3            |                                     |                                     |
|----|-------------------------------------|----------------|----------------------------|------------------------------------|------------------------|--------------------------------|-------------------|------------------|-------------------------------------|-------------------------------------|
|    |                                     | Percent $H_2O$ | Percent Available $P_2O_5$ | Percent Citrate Insoluble $P_2O_5$ | Percent Total $P_2O_5$ | Percent Water Soluble $P_2O_5$ | Percent Free Acid | Percent Fluorine | Percent Available of Total $P_2O_5$ | Percent Conversion of Rock $P_2O_5$ |
|    | Percent Available $P_2O_5$          | 42.9           | 47.9                       | 49.1                               |                        |                                |                   |                  |                                     |                                     |
|    | Percent Citrate Insoluble $P_2O_5$  | 4.5            | 1.9                        | 0.6                                |                        |                                |                   |                  |                                     |                                     |
|    | Percent Total $P_2O_5$              | 47.4           | 49.9                       | 49.6                               |                        |                                |                   |                  |                                     |                                     |
|    | Percent Water Soluble $P_2O_5$      | 40.1           | 45.1                       | 45.6                               |                        |                                |                   |                  |                                     |                                     |
|    | Percent Free Acid                   | 4.9            | 3.8                        | 4.9                                |                        |                                |                   |                  |                                     |                                     |
|    | Percent Fluorine                    | 1.1            | 0.8                        | 0.6                                |                        |                                |                   |                  |                                     |                                     |
| 35 | Percent Available of Total $P_2O_5$ | 90.5           | 96.1                       | 98.9                               |                        |                                |                   |                  |                                     |                                     |
|    | Percent Conversion of Rock $P_2O_5$ | 69.1           | 85.9                       | 95.6                               |                        |                                |                   |                  |                                     |                                     |

EXAMPLE II

Superphosphoric acid was heated in 100 ml. beakers on a hotplate to 300° F. The acid had a total of 71.05 weight percent of  $P_2O_5$ , 43.3% ortho and 0.17% insoluble  $P_2O_5$ . The hot acid was mixed with low grade phosphate rock at a  $P_2O_5/CaO$  ratio of 1.0. The rock was Bartow, Fla., phosphate rock having 0.1%  $H_2O$ , 40.15%  $CaO$ , 28.1%  $P_2O_5$  and 3.4% fluorine.

45 Three sets of the above samples were placed in ovens regulated to the following temperatures: 431° F., 345° F. and 277° F. After being heated for 30 minutes at the above temperatures, the samples were stored for nine days in the conventional triple superphosphate den for further reaction and at the end of nine days the triple superphosphate products analyzed as follows:

TABLE II

| Temp., ° F. | Percent $P_2O_5$ |       |        |            | Percent F. | Percent Free Acid | Percent Available of Total $P_2O_5$ | Percent Conversion of Rock $P_2O_5$ |
|-------------|------------------|-------|--------|------------|------------|-------------------|-------------------------------------|-------------------------------------|
|             | Total            | C. I. | Avail. | Water Sol. |            |                   |                                     |                                     |
| 277         | 51.9             | 3.8   | 48.2   | 47.5       | 0.99       | 8.0               | 92.8                                | 82.1                                |
| 345         | 52.2             | 3.6   | 48.5   | 47.5       | 0.83       | 8.3               | 93.1                                | 83.2                                |
| 431         | 52.7             | 3.7   | 49.0   | 45.4       | 0.74       | 7.3               | 93.0                                | 83.0                                |

the mixing operation may be carried on at room temperature, I prefer to heat the superphosphoric acid to temperatures above 100° F. and preferably to the temperature range of 250–450° F. If desired, the superphosphoric acid may be preliminarily heated to about 300° F. and low grade phosphate rock may be mixed with the hot acid preferably at a  $P_2O_5/CaO$  ratio of 1.0. Thereafter, the mixture may be heated, as by placing in ovens, to the higher range of temperatures preferably 250–450° F. and the heated mixture then stored in a den, say for about nine days, etc., to produce the triple superphosphate product.

While in the foregoing specification I have set forth specific embodiments of the invention in considerable detail for the purpose of illustrating the invention, it will be understood that such details may be varied widely by those skilled in the art without departing from the spirit of my invention.

I claim:

1. In a process for the manufacture of triple superphosphate, the steps of acidulating low-grade phosphate ore having less than 62 BPL, with wet process superphosphoric acid having at least 65 weight percent  $P_2O_5$  equivalent and at a  $P_2O_5/CaO$  ratio of about 1.0 to 1.1,

heating the same to a temperature in the range of about 250-450° F. and storing the heated mass for reaction to form triple superphosphate.

2. In a process for the manufacture of triple superphosphate, the steps of acidulating low-grade phosphate ore having a BPL less than 62 with wet process superphosphoric acid having in excess of 70 weight percent  $P_2O_5$  equivalent and at a  $P_2O_5/CaO$  ratio of about 1.0, heating the same to a temperature in the range of 250°-450° F. and storing the heated mass for reaction to form triple superphosphate. 5

3. In a process for the manufacture of triple superphosphate from low grade phosphate rock, the steps of mixing phosphate rock having a BPL below 62, with wet process superphosphoric acid of about 72 weight percent  $P_2O_5$  equivalent and a  $P_2O_5/CaO$  ratio of about 1.0, heating the mixture to a temperature of about 250°- 10

450° F. for a period of about 30 minutes, and then storing the heated mass in a den for reaction to form triple superphosphate.

#### References Cited

##### UNITED STATES PATENTS

|           |         |                  |        |
|-----------|---------|------------------|--------|
| 2,160,700 | 5/1939  | Knox             | 23—109 |
| 2,271,361 | 1/1942  | Carpenter et al. | 23—109 |
| 2,296,494 | 9/1942  | Block            | 23—109 |
| 2,296,495 | 9/1942  | Block            | 23—109 |
| 2,522,500 | 9/1950  | Bridger          | 71—41  |
| 3,212,874 | 10/1965 | Baumann          | 71—34  |

EARL C. THOMAS, Primary Examiner.

OSCAR R. VERTIZ, Examiner.

L. A. MARSH, Assistant Examiner.